

1,631,249

June 7, 1927.

C. L. CORFMAN

INVESTMENT COMPOSITION

Filed Dec. 30, 1925



Fig. 1



Fig. 2

Inventor  
Clifford L. Corfman

By *Herbert E. Smith*

Attorney

## UNITED STATES PATENT OFFICE.

CLIFFORD L. CORFMAN, OF SPOKANE, WASHINGTON.

## INVESTMENT COMPOSITION.

Application filed December 30, 1925. Serial No. 78,384.

The present invention relates to an improved investment composition especially adapted for use in dentistry. The composition or material is used in molds for the 5 investment of wax patterns for inlays, crowns, bridge work and similar dental appliances where heat is to be used for soldering and casting gold and other metals after the mold has been prepared.

10 According to well known dental practice, after the wax impression is made, mounted upon its stem and attached to its base member, the whole is invested in material within a mold and the base and stem and wax impression subsequently removed, after which the mold may be baked to eliminate moisture and prepare the mold for casting. After casting the investment material is broken away, and the casting should be 20 ready for use after polishing.

Plaster of Paris is the customary material utilized for investment purposes, and I am aware that it has been proposed to use compositions or compounds which include 25 other elements or ingredients in the material. With all such materials difficulty is encountered and imperfect patterns result from expansion and contraction of the investment material or mold, and consequently inaccuracies and imperfections follow in the casting or soldering operations, necessitating tedious and expensive work on the appliance 30 before it can be put into use.

I have found that by the use of magnesite 35 in combination with the plaster of Paris in the approximate proportions of two to one furnishes an investment material from which the moisture may thoroughly and with rapidity be eliminated from the matrix 40 or mold and the latter is not subjected to perceptible contraction or expansion, thereby insuring accuracy in casting and soldering operations; smooth surfaces are provided on the mold to which the cast metal will not 45 adhere and therefore imperfections or irregularities do not appear on the finished article, and the article or appliance is not subject to contamination from the investment material.

In order that the invention may readily 50 be understood I have illustrated in the accompanying drawings a matrix or mold in which the investment material is made according to my invention.

Figure 1 is a sectional view of the matrix 55 or mold showing the wax impression and stem with its base in the material.

Figure 2 is a view of the matrix ready for pouring or casting.

A well known type of cylindrical shell 1 60 is utilized and upon the base 2 the wax stem 3 is built for supporting the wax impression 4 secured in usual manner. The investment material is indicated as 5 and is placed in the shell in plastic condition as 65 usual. After the base 2 has been removed the wax stem and impression may be melted in usual manner and removed, after which the matrix is baked or otherwise dried and the molten metal, as gold is poured into the 70 opening 6.

In forming the investment material I use approximately one part of plaster of Paris and two parts of magnesite. The plaster of Paris is of course finely ground, and the 75 magnesite is dead burned and finely pulverized. The magnesite, which is a soft white mineral forms a base for the plaster of Paris which readily compounds with the base in the presence of a sufficient quantity 80 of moisture for the purpose. The plaster of Paris and magnesite are thoroughly intermingled and intimately mixed to form a plastic composition of the desired consistency for properly investing the wax impression as indicated in Figure 1. The plastic mixture is capable of being solidly compacted to closely invest the core or wax members, and after the base has been removed 85 and the material set, the matrix is baked or otherwise dried to remove moisture leaving a solid and substantial mold for the reception of the molten metal poured into the opening 6.

While the mold is hard and solid, it may yet readily be broken away from the crown, bridge or other accessory of the dental art that is cast in the matrix and the material 90

can be thoroughly removed from the accessory with convenience and facility leaving only a slight touching up or polishing of the crown in its finished or completed form.

5 Having thus fully described my invention, what I claim as new and desire to secure by Letters Patent is—

1. An investment composition for dental

use comprising magnesite as a base and plaster of Paris.

10 2. An investment composition comprising approximately two parts magnesite and one part plaster of Paris.

In testimony whereof I affix my signature.

CLIFFORD L. CORFMAN.